

1

3,231,372

## MAGNESIUM-BASE ALLOYS CONTAINING RARE EARTH METALS

George S. Foerster, Midland, Mich., assignor to The Dow Chemical Company, Midland, Mich., a corporation of Delaware  
No Drawing. Filed Sept. 27, 1963, Ser. No. 311,997  
6 Claims. (Cl. 75—168)

This invention relates to magnesium-base alloys containing rare earth metals having improved strength properties.

Though magnesium-base alloys containing various rare earth metal mixtures such as, for example, misch metal and didymium retain a higher proportion of their physical properties at elevated temperatures than other magnesium-base alloys, they tend to have low strength at room temperatures, and thus, correspondingly lower strength properties at elevated temperatures, especially when extruded at either high temperatures or at high speeds.

An object of the present invention, therefore, is to provide a magnesium-base alloy containing rare earth metal having improved physical properties at normal ambient or room temperatures. A related object is to provide such an alloy whose properties are also improved at elevated temperatures.

The term "rare earth metal" as used herein refers to the metals, either singly or mixtures thereof, having atomic numbers from 57 to 71, inclusive, commonly referred to as those in the lanthanide series.

The above object and other objects and advantages of the invention have surprisingly and unexpectedly been found obtainable in a magnesium-base alloy containing rare earth metals by adding particular amounts of aluminum thereto relative to the amount of rare earth metal present in the alloy.

Accordingly, the alloy of the present invention consists of a magnesium-base alloy comprising an amount within the range of from about 0.2 to about 4.0 weight percent of a rare earth metal such as, preferably for example, lanthanum, praseodymium, neodymium, or cerium, or a mixture of rare earth metal such as, for example, misch-metal (MM) or didymium (Di), and an amount of aluminum within the range of from 0.05 to about 0.8 percent by weight.

Optimum room temperature properties are obtained in the alloy where the rare earth metal content is within the range of from about 0.5 to about 2.0 weight percent,

2

in that the aluminum content should not at any time exceed the rare earth content and as the amount of rare earth metal used is increased so also is the amount of aluminum. For example, when 0.5 percent misch metal is employed, the aluminum content may be about 0.2 percent; whereas when about 1 percent didymium is present about 0.4 percent of aluminum may be employed; and at 2 percent didymium, about 0.6 percent aluminum is indicated.

Small amounts of manganese may also be employed in the magnesium-base alloy of the present invention for enhanced properties within the range of from about 0.1 to about 0.6.

Improvement of the properties of the magnesium-base rare earth metal system, particularly in strength, is unexpected inasmuch as aluminum added to such a system is normally deleterious. Surprisingly, however, it has been found that the addition of aluminum to such a system with the range of aforesaid and in accordance with the present invention is not deleterious but in fact remarkably improves the room temperature properties of the alloy and its properties at elevated temperatures.

The following examples serve to further illustrate the present invention.

Various alloys in accordance with the present invention and others for comparison as blanks were made using conventional alloying and melting techniques as practiced in the magnesium art, each having the composition indicated in Table 1. These alloys were cast into billets which were subsequently extruded from a 3 inch container of a ram extrusion machine at the speeds indicated into  $\frac{1}{16}$  inch by  $\frac{1}{8}$  inch strips, at a temperature of about 750° F., followed by aging for about 24 hours at a temperature within the range of from about 350° F. to about 400° F.

The so-prepared strips, as indicated in Table 1, were then tested at room temperature (25° to 28° C.) for percent elongation (percent E) (using a 2 inch gauge length), tensile yield strength (TYS) (at a 0.2 percent deviation from the modulus line), compression yield strength (CYS), and tensile strength (TS). The results of these tests under the conditions indicated are shown in Table 1. Examples 1 and 2 therein were aged at about 350° F., 3 and 4 at 375° F., and 5 and 6 at 400° F.

It should be understood that other fabrication means and ageing conditions, including heat treatments, than those employed above can be used with respect to the alloys of the present invention in order to obtain other and varied properties in said alloys.

Table 1

| Example | Magnesium-Base Plus |            |           |            | Extrusion Speed f.p.m. <sup>1</sup> | Percent E | 1,000 p.s.i. <sup>2</sup> |     |    | Extrusion Speed f.p.m. <sup>1</sup> | Percent E | 1,000 p.s.i. <sup>2</sup> |     |    |
|---------|---------------------|------------|-----------|------------|-------------------------------------|-----------|---------------------------|-----|----|-------------------------------------|-----------|---------------------------|-----|----|
|         | Percent Di          | Percent MM | Other, Mn | Percent Al |                                     |           | TYS                       | CYS | TS |                                     |           | TYS                       | CYS | TS |
| Blank   |                     | 0.5        | 0.5       |            | 20                                  | 21        | 14                        | 12  | 30 | 100                                 | 12        | 18                        | 11  | 35 |
| (1)     |                     | 0.5        | 0.5       | 0.2        | 20                                  | 16        | 26                        | 19  | 38 | 100                                 | 14        | 23                        | 14  | 37 |
| (2)     |                     | 0.5        | 0.5       | 0.4        | 20                                  | 6         | 28                        | 12  | 40 | 100                                 | 6         | 30                        | 12  | 42 |
| Blank   | 1.0                 |            |           |            | 10                                  | 28        | 14                        | 15  | 33 | 50                                  | 20        | 12                        | 13  | 35 |
| (3)     | 1.0                 |            |           | 0.4        | 10                                  | 14        | 28                        | 26  | 38 | 50                                  | 14        | 28                        | 21  | 39 |
| (4)     | 1.0                 |            |           | 0.8        | 10                                  | 8         | 27                        | 14  | 40 | 90                                  | 9         | 28                        | 14  | 40 |
| Blank   | 2.0                 |            |           |            | 10                                  | 24        | 14                        | 14  | 35 | 25                                  | 30        | 12                        | 13  | 37 |
| (5)     | 2.0                 |            |           | 0.2        | 10                                  | 24        | 22                        | 20  | 36 | 30                                  | 24        | 17                        | 17  | 38 |
| (6)     | 2.0                 |            |           | 0.8        | 10                                  | 36        | 25                        | 41  |    | 50                                  | 10        | 30                        | 16  | 41 |

<sup>1</sup> F.p.m.=feet per minute.

<sup>2</sup> P.s.i.=pounds per square inch.

and the amount of aluminum is from about 0.2 to about 0.6 weight percent.

It is preferable to gauge the amount of aluminum in the alloy in accordance with the amount of rare earth

From the figures in the examples given in Table 1 above compared to those for the blanks, the improved strength properties of the alloys representative of the present invention are clearly illustrated.

Among the advantages of the alloy are that it has the light weight characteristic of magnesium, and a high strength to weight ratio, particularly at elevated temperatures and is composed of relatively small amounts of metals, those most preferred being readily available.

The term "magnesium" as used herein refers to the pure and commercial metal having less than about 0.3 percent of other constituents therein either as additives or as unavoidable impurities.

What is claimed and desired to be secured by Letters Patent is:

1. A magnesium-base alloy consisting essentially of rare earth metal in an amount by weight within the range of from about 0.2 to about 4.0 percent, and aluminum in an amount by weight within the range of from about 0.05 to about 0.8 percent, the balance being essentially magnesium, with the amount of aluminum employed not exceeding that of the rare earth metal.

2. The magnesium-base alloy of claim 1 wherein the rare earth metal is one selected from the group consisting of lanthanum, praseodymium, neodymium, and cerium.

3. The magnesium-base alloy of claim 1 wherein the rare earth metal is present in an amount by weight within the range of from about 0.5 to about 2.0 percent and aluminum is in an amount within the range of from about 0.2 to about 0.6 percent.

4. The magnesium-base alloy of claim 3 wherein the rare earth metal employed is misch metal.

5. The magnesium-base alloy of claim 3 wherein the rare earth metal employed is didymium.

6. The magnesium-base alloy of claim 1 including an amount of manganese within the range of from about 0.1 to about 0.6.

#### References Cited by the Examiner

##### UNITED STATES PATENTS

2,221,319 11/1940 Altwicker et al. \_\_\_\_\_ 75—168

2,801,166 8/1957 Lucien et al. \_\_\_\_\_ 75—168

20 DAVID L. RECK, *Primary Examiner.*